

## UNITED STATES PATENT OFFICE

RALPH W. FREY, OF MOUNT RAINIER, MARYLAND, ASSIGNOR TO THE GOVERNMENT  
AND THE PEOPLE OF THE UNITED STATES OF AMERICA

## TANNING PREPARATION AND PROCESS

No Drawing. Original application filed April 28, 1927, Serial No. 187,418. Divided and this application filed July 31, 1928. Serial No. 296,623.

(GRANTED UNDER THE ACT OF MARCH 3, 1883, AS AMENDED APRIL 30, 1928; 370 O. G. 757)

This invention is made under the act approved April 30, 1928, and the invention herein described, if patented, may be manufactured and used by or for the Government for governmental purposes without payment to me of any royalty thereon. I hereby dedicate the invention herein described to the free use of the public, to take effect upon the granting of a patent to me.

10 This application is a divisional application of my application for patent which bears Serial No. 187,418, filed April 28, 1927, on tanning preparations and processes.

15 According to my invention tanning preparations, in either liquid or solid form, are produced from chromium and iron. These preparations can be used for tanning with both the chromium salts and iron salts present, the two tanning principles acting either simultaneously or successively, or, if desired, these preparations, without removal of the iron salts, can be used for tanning with the chromium salts only, producing a leather of 20 normal chrome "crust" color and of a better than normal substance, particularly in the loose and more flabby parts of the hide or skin. The production of such leather in the presence of relatively high percentage of 25 iron salts in a non-tanning state is also a novel feature of my invention.

While metallic chromium and metallic iron are available in several forms, a particularly convenient and economical commercial source 30 is the alloy known as ferro-chrome. Ferro-chrome is readily available in large quantities. Its composition can be controlled to produce, from a raw material standpoint, a product of unusual physical and chemical 35 uniformity. It has a further advantage for tanning in that the chromium predominates over the iron.

40 Ferro-chrome alloys are divided into two classes, high-carbon ferro-chrome and low-carbon ferro-chrome. While either may be used, low-carbon ferro-chrome alloys are not to be preferred as they are relatively higher priced and also are needlessly refined with respect to the removal of carbon.

50 The percentage composition range for a

good grade of high-carbon ferro-chrome may be represented as follows:

|                           |           |    |
|---------------------------|-----------|----|
| Cr                        | 60 to 70% | 60 |
| Fe                        | 20 to 30% | 55 |
| C                         | 4 to 6%   | 65 |
| Si and other constituents | 1 to 2%   | 60 |

It will thus be seen that ferro-chrome is extremely rich in chromium and iron.

According to my invention chromium and iron are dissolved in water and hydrochloric acid in suitable proportions. Hydrochloric acid is particularly advantageous under some conditions of tanning because the chlorides of iron are less prone to hydrolysis and precipitation than are the sulphates prepared in a similar way as described in my application Serial No. 187,418.

After the metals have been dissolved the 70 solution is neutralized to the extent desired depending upon the basicity required by a particular stock and process. Various well-known neutralizing agents such as the oxides, hydroxides, carbonates, borates, phosphates, 75 and acetates of the alkalis and alkali-earths may be used, the selection of the neutralizing agent depending largely upon the desired properties of the leather.

After partial neutralization the solution is 80 ready for immediate use or it may be evaporated to dryness or other degree of concentration for storage or shipment.

Simply as an illustration of the preparation of such a stock tanning solution, but in no sense a restriction as to the kind and quantity of materials, the following example is offered:

Example 1.—To one part by weight of ferro-chrome alloy add a mixture of from 90 five to seven parts by weight of water and from five to six parts by weight of 20° to 22° Bé. hydrochloric acid. After the reaction subsides boil gently until the ferro-chrome is dissolved, keeping the original volume about 95 constant, then determine the Fe, Cr, and titratable Cl in the solution. From these data calculate the Cl equivalent to the Fe as  $FeCl_2$ ; the Cl equivalent to the Cr as  $CrCl_3$ , and the "free" or excess Cl. Ignore the Cl 100

of the  $\text{FeCl}_2$  and calculate the quantity of  $\text{Na}_2\text{CO}_3$  necessary to neutralize all of the excess Cl and also that proportion of the Cl associated with the chromium to give the desired basicity or degree of neutralization. 5 The most suitable basicity must be determined for the particular conditions of use. Dissolve the required quantity of  $\text{Na}_2\text{CO}_3$  in water and add it to the ferro-chrome solution slowly while stirring vigorously. The resulting solution is then ready for tanning.

10 In the tanning preparation such as described the chromium salts and iron salts are in the reduced state, in which state the chromium tans whereas the iron does not. As a consequence, and if desired, chrome tanning can be carried on without any iron tanning. For such a process the hides or skins after coming out of the customary foretanning operations such as liming, unhairing, deliming, and pickling, are started in the tanning operation proper with the stock iron-chromium solution in the same manner that an ordinary stock chrome solution is used, the necessary 15 quantity of stock iron-chromium solution being based on its  $\text{Cr}_2\text{O}_3$  content and the weight of the hides or skins. When the last half of the tanning operation is reached a neutralizing agent such, for example, as  $\text{NaHCO}_3$  is 20 added to just short of the precipitation point of the liquor and the tanning is continued until the leather responds properly to the boiling water test. At this stage, or after "horsing", the leather is washed free of iron 25 salts. The remaining operations, including the final neutralization of the leather, are carried out in the usual manner.

30 By such a process a chrome tanned leather of a normal chrome "crust" color is obtained in the presence of material quantities of iron salts in a non-tanning state. While the iron salts do not enter into the tanning and thus color the leather their presence in the liquor results in a chrome tanned leather of more 35 than the customary "fullness" or substance, especially in the naturally flabbier parts of the hide or skin.

40 Iron-chromium preparations such as described can also be used to carry on a joint chrome-iron tannage with the production of leathers of unique and desirable properties. For such a joint tannage the iron in the solution is oxidized to the ferric or tanning state by suitable means either before the tanning 45 operation proper is started or later on after the chrome tanning has been partially or entirely completed.

50 Various oxidizing agents can be used. So sodium dichromate has, however, several advantages in that the oxidation of the iron is readily carried to completion at ordinary temperatures and the chromium reduced thereby from the dichromate becomes available as additional tanning material. The re-

action may be represented by the following well-known equations:



70 As shown, the reaction reduces the acidity of the tanning liquor. Consequently in tanning a further neutralization of the liquor, which is often practiced in ordinary mineral tanning, is not necessary.

75 As an illustration of a procedure for a joint chromium-iron tannage the following example is offered.

80 *Example 2.*—Using a stock ferro-chrome alloy solution such as described in Example 1, the first stages of the tanning operation proper are carried out in the same manner as for ordinary stock chrome solutions, except that the quantity of stock ferro-chrome alloy solution to be used as based on its  $\text{Cr}_2\text{O}_3$  content and the weight of the hides or skins can be less than the customary quantity because of the subsequent tanning action of the iron present. This reduction may be from 85 15 to 25 per cent of the allowance of  $\text{Cr}_2\text{O}_3$  for ordinary stock chrome solutions. After all of the stock ferro-chrome solution has been added and the tanning is about half completed  $\text{Na}_2\text{Cr}_2\text{O}_7 \cdot 2\text{H}_2\text{O}$ , dissolved in water, is 90 slowly added with motion and while the tanning is being continued. The required quantity of  $\text{Na}_2\text{Cr}_2\text{O}_7 \cdot 2\text{H}_2\text{O}$  is determined from the calculated  $\text{FeCl}_2$  content of the ferro-chrome solution used, by means of the oxidation equation already given. The tanning is then continued until the desired degree of 95 joint chromium-iron tannage is obtained, after which the leather is washed, neutralized, and finished as is customary.

100 Such a tannage proceeds very smoothly and the leathers produced thereby are of excellent quality, having an unusual "fullness" and are soft and pliable. They show none of the undesirable properties such as flatness, tinniness, harshness, brittleness, and 105 weak fiber, that have generally resulted from previous attempts to produce leathers of an entire or partial iron tannage. They have an attractive natural light buff to tan color that is suitable for many purposes, thus making unnecessary extra dyeing operations. The natural color being mineral in nature and being all through the leather as well as on its surfaces, is unusually permanent.

110 I claim:

1. The process of making a tanning preparation which consists in dissolving chromium and iron in hydrochloric acid and water and rendering the resulting solution basic by the 115 addition of an alkali carbonate.
2. The process of making a tanning preparation which consists in dissolving an alloy of chromium and iron in hydrochloric acid and water and rendering the resulting solu- 120 130

tion basic by the addition of an alkali carbonate.

3. The process of making a tanning preparation which consists in dissolving ferro-chrome in hydrochloric acid and water and rendering the resulting solution basic by the addition of an alkali carbonate.

5 4. The process of making a tanning preparation which consists in dissolving chromium 10 and iron in hydrochloric acid and water, then rendering the resulting solution basic by the addition of an alkali carbonate, and oxidizing the iron salts present to the ferric state by the addition of an alkali dichromate.

15 5. The process of making a tanning preparation which consists in dissolving an alloy 20 of chromium and iron in hydrochloric acid and water, then rendering the resulting solution basic by the addition of an alkali carbonate, and oxidizing the iron salts present to the ferric state by the addition of an alkali dichromate.

25 6. The process of making a tanning preparation which consists in dissolving ferro-chrome in hydrochloric acid and water, then 30 rendering the resulting solution basic by the addition of an alkali carbonate, and oxidizing the iron salts present to the ferric state by the addition of an alkali dichromate.

35 7. A chrome tanning preparation comprising 40 a solution of chromium and iron in hydrochloric acid and water, which solution has been rendered basic.

8. A chrome tanning preparation comprising 45 a solution of ferro-chrome in hydrochloric acid and water, which solution has been rendered basic.

9. The step in the process of making 50 chrome leather comprising the tanning of 40 hides and skins with a solution of chromium and iron dissolved in hydrochloric acid and water and rendered basic.

10. The step in the process of making 55 chrome leather comprising the tanning of 45 hides and skins with a solution of ferro-chrome dissolved in hydrochloric acid and water and rendered basic.

11. The steps in the process of making 60 chrome-iron leather comprising the tanning 50 of hides and skins with a solution of chromium and iron dissolved in hydrochloric acid and water and rendered basic, followed during the tanning by the addition to the solution of an oxidizing agent to oxidize the iron 55 salts present to the ferric state.

12. The steps in the process of making 65 chrome-iron leather comprising the tanning 55 of hides and skins with a solution of ferro-chrome dissolved in hydrochloric acid and 80 water and rendered basic, followed during the tanning by the addition to the solution of an oxidizing agent to oxidize the iron salts present to the ferric state.

RALPH W. FREY.